

## UNITED STATES PATENT OFFICE

1,968,344

## MAILLEABLE ALUMINUM ALLOY

Karl Leo Meissner, Duren, Germany, assignor of one-half to the firm Dürener Metallwerke Aktiengesellschaft, Duren, Germany, a joint-stock company of Germany

No Drawing. Application August 31, 1932, Serial No. 631,301. In Germany September 12, 1931

## 3 Claims. (Cl. 75—1)

This invention relates to malleable and age-hardenable aluminum alloys.

In the employment of aluminum alloys, above all for vehicular construction, and especially in aircraft construction, the constant endeavour, since the invention of the age-hardenable aluminum alloys, has been to improve still further the mechanical properties of these alloys, with a view to lowering the dead weight of the structures. In so doing, importance has been attached, not only to increasing the tensile strength, but also, in particular, to increasing the elastic limit and yield point, which constitutes a factor of almost greater importance. Although it was possible without difficulty to raise the yield point and tensile strength of the aluminum alloys known in the art, by cold working, this treatment could be only applied to a certain extent, since otherwise, other valuable properties such as elongation and capacity for cold working would be too adversely affected thereby. On this account it became necessary to discover alloys endowed, from the outset, with greater strength coupled with satisfactory values with respect to elongation and capacity for cold working.

25 Exhaustive experiments have now shown that specially high qualities are possessed by aluminum alloys of the following composition:—

|                     | Per cent   |
|---------------------|------------|
| Copper              | 3 to 5     |
| Magnesium           | 0.7 to 1.2 |
| Silicon             | 0.4 to 0.7 |
| Manganese           | 0.6 to 1.4 |
| Remainder aluminum. |            |

35 Alloys of this composition are still suitably malleable, both in the hot and in the cold states.

For example, an alloy containing 4.0% of copper, 1.0% of magnesium, 0.58% of silicon and 1.2% of manganese, exhibits a yield point of about 16 to 17 kgs. per sq. mm., a tensile strength of 36 to 37 kgs. per sq. mm. and an elongation of 21 to 22%, immediately after quenching from the high temperature treatment. After aging several days at ordinary temperatures, such an alloy attains mechanical properties hitherto un-

obtainable, namely, yield points of about 31 to 33 kgs. per sq. mm. and tensile strengths of 48 to 50 kgs. per sq. mm., the elongation receding to about 18 to 20 per cent.

Another alloy, containing 4.0% of copper, 1.2% of magnesium, 0.7% of silicon and 1.2% of manganese, exhibits, immediately after quenching from the high temperature treatment, tensile values regarded as normal in the case of the previously known alloys when in the fully age-hardened state. The tensile strength of this alloy is already 37 to 39 kgs. per sq. mm., and the elongation about 20 to 21%. At the same time, however, the yield point of about 19 to 20 kgs. per sq. mm., is still lower than that of the hitherto known alloys after aging. After being kept for several days at room temperature, this alloy also attains a yield point of about 31 to 33 kgs. per sq. mm., and tensile strengths of 48 to 50 kgs. per sq. mm., whereas the elongation diminishes again, namely to 18 to 19%.

As is clear from the above examples the magnesium and silicon must be so proportioned that they are present almost wholly in the form of the compound magnesium silicide without an excess of either free magnesium or free silicon.

I claim:—

1. A malleable aluminum alloy which consists of about 4% of copper, about 1% of magnesium, about 0.58% of silicon, and about 1.2% of manganese, the remainder being aluminum.

2. A malleable aluminum alloy which consists of about 4% copper, about 1.2% of magnesium, about 0.7% of silicon, and about 1.2% of manganese, the remainder being aluminum.

3. A malleable aluminum alloy which consists of aluminum with 3 to 5% of copper, 0.6 to 1.4% of manganese, 0.7 to 1.2% of magnesium, and 0.4 to 0.7% of silicon, the latter two components being so proportioned that they are present almost wholly in the form of the compound magnesium silicide without leaving either free magnesium or silicon.

KARL LEO MEISSNER.